

June 24, 1958

E. C. OKRESS ET AL

2,840,493

METHOD OF EMISSION SUPPRESSION IN VACUUM  
TUBES, ESPECIALLY MAGNETRON HATS

Filed Nov. 22, 1952



Fig. 1.



Fig. 2.



Fig. 3.

WITNESSES:

John E. Heasley  
Leon M. Garman

INVENTORS  
Ernest C. Okress &  
Ralph J. Green

BY

J. E. Browder  
ATTORNEY

1

2,840,493

**METHOD OF EMISSION SUPPRESSION IN VACUUM TUBES, ESPECIALLY MAGNETRON HATS**

Ernest C. Okress, Montclair, and Ralph J. Green, Newark, N. J., assignors to Westinghouse Electric Corporation, East Pittsburgh, Pa., a corporation of Pennsylvania

Application November 22, 1952, Serial No. 321,976

2 Claims. (Cl. 117—216)

Our invention relates to graphite and metal-coatings and in particular relates to methods of applying coatings to surfaces of metallic structural elements in electrical discharge devices to decrease their electron emission and simultaneously to increase thermal emissivity.

As is more fully described in application Serial No. 319,032, now Patent No. 2,631,047, of Ernest E. Okress for "Cathode End-Shields for Magnetrons," filed concurrently herewith, certain structural elements supported at the ends of the cylindrical hat-cathodes in present-day magnetrons tend to become thermionically or secondarily emissive of their own accord or due to the contaminants thereon while the magnetrons are operating and to cause injurious arc-overs under the electric field-stresses existing in their vicinity. The said application describes and claims, among other things, the expedient of coating such structural elements with graphite to prevent such arcing.

While the coatings described in the Okress application have been found satisfactory in most conditions of operation, it has been found that in tubes operating under conditions of extra high voltage-stress, any loosely deposited carbon is likely to be dislodged with consequent loss of effectiveness and may initiate arcing. While deposition of a more adherent carbon, namely graphite, by pyrolysis of hydrocarbons at more elevated temperatures is possible, such coatings have proven much less effective than is required in preventing electron emissions when using black sooty carbon.

One object of our invention is accordingly to provide a way of forming on metallic surfaces a carbon coating which is permanently adherent while at the same time efficient in preventing electron emission from causes referred to above.

Another object is to provide metallic surfaces with a carbon coating which is firmly adherent while at the same time having a high thermal emissivity.

Yet another object is to provide a method of coating metal surfaces with a firmly adherent coating of material which has low electron emission characteristics.

Still another object is to provide a method of coating metal surfaces with a firmly adherent layer of low electron-emission characteristics of zirconium, zirconium oxide or other electron-suppressive materials.

A further object is to provide a method of producing a porous surface on metals, such for example as tantalum.

Yet another object is to provide an improved surface for electrodes or other structures subject to high electric gradients.

Other objects of our invention will become apparent upon reading the following description taken in connection with the drawings in which:

Figure 1 is a schematic view indicating the porous structure of a metallic base-material used to fabricate electron tube electrodes and other structural elements in accordance with our invention;

Fig. 2 is a view partly in section of a magnetron

2

cathode provided with an end-shield made in accordance with our invention;

Fig. 3 is a diametral section of one form of the metallic base used in forming the end-shield.

As has been briefly stated above, difficulty is found in electron tube practice from the tendency of metal structures within the tube to emit electrons at undesired places which may produce a variety of undesirable effects such, for example, as arc-overs and insulation failures. Such electrons may, in the case of unheated structural elements, be due to secondary electron emission of the base metal itself or the active contaminants deposited thereon during normal operation. These contaminants normally come from the heated active cathode surface.

The cause of this spurious emission is electron and ion bombardment and X-ray photo-induced. In the case of structures intentionally heated, or those unavoidably heated by proximity to neighboring elements, the emission may be thermionic as well. As is disclosed and claimed in the Okress application previously mentioned, such electron-emission may be minimized by coating the metallic structures with a layer of graphite or certain other electron-suppressive and heat dissipative materials. In accordance with our present invention, superior coatings of this kind may be formed by making the underlying metal porous as indicated in Fig. 1, where the metal particles or crystals 1 are separated from each other by pores 2. The electron suppressive coating 3 may be graphite, zirconium, zirconium oxide or other emission-suppressive and heat-dissipative material.

The porous underbody of metal may be formed in several different ways. A widely used metal for high voltage electron-tube electrode-supports and the like is tantalum, and one method of forming the desired porous surface is to mold the structural element from powdered tantalum, as shown in Fig. 3, in a press and sinter the resulting structure at a temperature sufficiently below the melting point so that the metal particles cohere but do not fully coalesce, as is known in the metallurgical art. This method is of course applicable to many metals besides tantalum; e. g. to nickel, tungsten and molybdenum which are frequently used in electron tube construction.

Another method of forming metallic members of porous structure is molding them from unstable compounds of the metal, followed by subsequent thermal or other decomposition of the compound. Tantalum chloride and iodide are such decomposable compounds of tantalum, for example.

Still another method of forming metallic members with porous surfaces is molding them with small percentages of these unstable metal compounds, organic chemical compounds, or combinations of the two followed by subsequent thermal decomposition of the compounds. For example, camphor and naphthalene are such decomposable organic chemical compounds.

However, the method which we have so far found most satisfactory for most purposes in forming porous-surface metals is to mold them from a powdered mixture of the tantalum or other desired structural metal with a small percentage of a metal having a lower melting point or high vapor-pressure which does not alloy readily with it. While in many structures it will be desirable to thus mold the entire structure desired, the covering of a non-porous metal core with a coating of the aforesaid mixture by spraying, on a metal base as shown in Fig. 2, or compressing it to form, as shewn in Fig. 3, are within the contemplation of our invention. To give one instance, tantalum powder may be mixed with five to ten percent of powdered nickel to carry out the foregoing procedure.

After thus shaping the structural element, it may be

heated beyond the melting point, or beyond the vaporizing point of the ancillary material, preferably in vacuum. This will leave the pores 2 of Fig. 1 between the metal particles 1.

The electron-suppressive coating 3 may be applied in one of several ways. For materials like zirconium, it may be produced by condensation on the cooled metal surface of zirconium vapor subliming from a body of that metal heated in vacuum. A carbon coating may be formed by pyrolysis through heating the porous metal in an atmosphere of hydrocarbon vapor, e. g., heating the metal to 1500 to 1600° C. in an atmosphere of benzene. In many cases we have found that the structure thus coated may be outgassed, carbon coated and again outgassed at a pressure of  $10^{-7}$  mm. of mercury in a single pumping operation.

Fig. 2 shows an example of a structural element formed in accordance with our invention, an end-shield 11 in position on the cathode 12 of a magnetron. The cathode 12 has a thermionically-emissive surface 13 supported on a hollow sleeve or core 14 with provisions for heating surface 13. An anode structure 15 surrounds the cathode 12 leaving an annular end-chamber 16 from which it is desirable to prevent electrons emitted by the surface 13. The end-shield 11, maintained substantially at the potential of cathode-surface 13, cooperates with anode 15 to produce an electric field which confines electrons, due to contamination of the surface 11 and its temperature, to the annular space 24. Unfortunately it often becomes a source of thermionic and secondary electrons in high-voltage magnetrons, and so to facilitate arc-overs to the anode which are fatal to successful operation.

Such undesired electron-emission from end-shield 11 may be minimized, as pointed out in the Okress application mentioned above, by covering the major portion of the surface of end-shield 11 with a coating 17 of electron-suppressive material such as graphite. To make this coating more effective and permanent, the main body 18 of the end-shield 11 is formed of porous metal such as sintered tantalum powders, formed as described in connection with Fig. 1. The end shield 11 is attached to the cathode-sleeve 14 by an uncoated portion 21 of the base metal 18 to which it may be attached by various methods. To minimize heat flow from the cathode-sleeve when this is at a higher temperature than the end sleeve 11, holes 23, spaced as closely together as is con-

sistent with mechanical strength, are formed in the shell 18 around its line of attachment to sleeve 14.

We claim as our invention:

5 1. The method of forming an electron-emission-suppressive surface on a refractory metal base member, said refractory metal being selected from the group consisting of tantalum, tungsten and molybdenum, said method including the steps of forming a non-porous surface layer of said refractory metal admixed with from 5 to 10% of a non-alloying material having a substantially higher vapor pressure than said refractory metal, said non-alloying material being selected from the group consisting of nickel, tantalum chloride, tantalum iodide, naphthalene and camphor, heating said surface layer until a substantial portion of said non-alloying material is removed from said surface layer thereby forming a porous surface layer of approximately 5 to 10% porosity, and coating said porous surface layer with a continuous layer of low electron-emissive material selected from the group consisting of graphite, zirconium and zirconium oxide.

20 2. The method of forming an electron-emission-suppressive surface on a tantalum base member, said method including the steps of forming a non-porous surface layer of tantalum admixed with from 5 to 10% nickel, heating said surface layer until a substantial portion of nickel is removed from said surface layer thereby forming a porous surface layer of approximately 5 to 10% porosity, and coating said porous surface layer with a continuous layer of low electron-emissive material selected from the group consisting of graphite, zirconium and zirconium oxide.

#### References Cited in the file of this patent

#### UNITED STATES PATENTS

|    |           |            |               |
|----|-----------|------------|---------------|
| 35 | 927,935   | Von Bolton | July 13, 1900 |
|    | 1,852,865 | Upp        | Apr. 5, 1932  |
|    | 1,985,087 | Glaser     | Dec. 18, 1934 |
|    | 2,149,657 | Armstrong  | Mar. 7, 1939  |
|    | 2,172,207 | Kolligs    | Sept. 5, 1939 |
| 40 | 2,251,410 | Koehring   | Aug. 5, 1941  |
|    | 2,348,045 | Wooten     | May 2, 1944   |
|    | 2,359,970 | Clark      | Oct. 10, 1944 |
|    | 2,417,730 | Becker     | Mar. 18, 1947 |
| 45 | 2,491,284 | Sears      | Dec. 13, 1949 |
|    | 2,497,109 | Williams   | Feb. 14, 1950 |
|    | 2,683,671 | Findlay    | July 13, 1954 |
|    | 2,687,466 | Mott       | Aug. 24, 1954 |